



US006444386B1

(12) **United States Patent**  
Liu et al.

(10) **Patent No.:** US 6,444,386 B1  
(45) **Date of Patent:** Sep. 3, 2002

(54) **PHOTOCONDUCTIVE IMAGING MEMBERS**

(75) Inventors: **Ping Liu; Cheng-Kuo Hsiao; Beng S. Ong**, all of Mississauga (CA); **Timothy J. Fuller; Huoy-Jen Yuh**, both of Pittsford, NY (US); **Helen R. Cherniack**, Rochester, NY (US); **Markus R. Silvestri**, Fairport, NY (US)

(73) Assignee: **Xerox Corporation**, Stamford, CT (US)

(\*) Notice: Subject to any disclaimer, the term of this patent is extended or adjusted under 35 U.S.C. 154(b) by 13 days.

(21) Appl. No.: **09/834,292**

(22) Filed: **Apr. 13, 2001**

(51) Int. Cl.<sup>7</sup> ..... **G03G 5/14**

(52) U.S. Cl. ..... **430/64**

(58) Field of Search ..... 430/64

(56) **References Cited**

U.S. PATENT DOCUMENTS

|             |         |                       |           |
|-------------|---------|-----------------------|-----------|
| 3,121,006 A | 2/1964  | Middleton et al. .... | 96/1      |
| 4,265,990 A | 5/1981  | Stolka et al. ....    | 430/59    |
| 4,298,697 A | 11/1981 | Baczek et al. ....    | 521/27    |
| 4,338,390 A | 7/1982  | Lu ....               | 430/106   |
| 4,464,450 A | 8/1984  | Teuscher ....         | 430/59    |
| 4,555,463 A | 11/1985 | Hor et al. ....       | 430/59    |
| 4,560,635 A | 12/1985 | Hoffend et al. ....   | 430/106.6 |
| 4,587,189 A | 5/1986  | Hor et al. ....       | 430/59    |
| 4,921,769 A | 5/1990  | Yuh et al. ....       | 430/64    |
| 4,921,773 A | 5/1990  | Melnik et al. ....    | 430/132   |

5,482,811 A 1/1996 Keoshkerian et al. .... 430/135  
6,287,737 B1 9/2001 Ong et al. .... 430/58.8

Primary Examiner—Mark Chapman

(74) Attorney, Agent, or Firm—E. D. Palazzo

(57)

**ABSTRACT**

A photoconductive imaging member containing a supporting substrate, a hole blocking layer thereover, a photogenerating layer, and a charge transport layer, and wherein the hole blocking layer is generated from crosslinking an organosilane (I) in the presence of a hydroxy-functionalized polymer (II)



for example, wherein R is alkyl or aryl, R<sup>1</sup>, R<sup>2</sup>, and R<sup>3</sup> are independently selected from the group consisting of alkoxy, aryloxy, acyloxy, halide, cyano, and amino; A and B are respectively divalent and trivalent repeating units of polymer (II); D is a divalent linkage; x and y represent the mole fractions of the repeating units of A and B, respectively, and wherein x is from about 0 to about 0.99, and y is from about 0.01 to about 1, and wherein the sum of x+y is equal to about 1.

**36 Claims, No Drawings**

## PHOTOCONDUCTIVE IMAGING MEMBERS

Illustrated in U.S. Pat. No. 6,287,737, the disclosure of which is totally incorporated herein by reference, is a photoconductive imaging member comprised of a supporting substrate, a hole blocking layer thereover, a photogenerating layer and a charge transport layer, and wherein the hole blocking layer is comprised of a crosslinked polymer generated, for example, from the reaction of a silyl-functionalized hydroxyalkyl polymer of Formula (I) with an organosilane of Formula (II) and water



wherein, for example, A, B, D, and F represent the segments of the polymer backbone; E is an electron transporting moiety; Z is selected from the group consisting of chloride, bromide, iodide, cyano, alkoxy, acyloxy, and aryloxy; a, b, c, and d are mole fractions of the repeating monomer units such that the sum of a+b+c+d is equal to 1; R is alkyl, substituted alkyl, aryl, or substituted aryl, with the substituent being halide, alkoxy, aryloxy, and amino; and R<sup>1</sup>, R<sup>2</sup>, and R<sup>3</sup> are independently selected from the group consisting of alkyl, aryl, alkoxy, aryloxy, acyloxy, haogen, cyano, and amino, subject to the provision that two of R<sup>1</sup>, R<sup>2</sup>, and R<sup>3</sup> are independently selected from the group consisting of alkoxy, aryloxy, acyloxy, and halide.

The appropriate components and processes of the above copending application may be selected for the present invention in embodiments thereof.

## BACKGROUND OF THE INVENTION

This invention is generally directed to imaging members, and more specifically, the present invention is directed to multilayered photoconductive imaging members with a hole blocking layer comprised of an interpenetrating polymer network comprised of a hydroxyfunctionalized polymer intertwined or intimately dispersed in with a crosslinked polysiloxane network derived from an organosilane reagent, such as alkoxy silane, amino alkyl alkoxy silane, acyloxy silane, cyanosilane, and the like, in the presence of an optional silane crosslinking catalyst of, for example, alkylamine or carboxylic acid. The hole blocking layer is preferably in contact with the supporting substrate and is preferably situated between the supporting substrate and the photogenerating layer, which is comprised of the photogenerating pigments of U.S. Pat. No. 5,482,811, the disclosure of which is totally incorporated herein by reference, especially Type V hydroxygallium phthalocyanine. The imaging members of the present invention in embodiments exhibit excellent cyclic/environmental stability, and substantially no adverse changes in their performance over extended time periods, since the imaging members comprise a mechanically robust and solvent resistant hole blocking layer, enabling the coating of a subsequent photogenerating layer thereon without structural damage, and which blocking layer can be easily coated on the supporting substrate by various coating techniques of, for example, dip or slot-coating. The aforementioned photoresponsive, or photoconductive imag-

ing members can be negatively charged when the photogenerating layers are situated between the hole transport layer and the hole blocking layer deposited on the substrate.

Processes of imaging, especially xerographic imaging and printing, including digital, are also encompassed by the present invention. More specifically, the layered photoconductive imaging members of the present invention can be selected for a number of different known imaging and printing processes including, for example, electrophotographic imaging processes, especially xerographic imaging and printing processes wherein charged latent images are rendered visible with toner compositions of an appropriate charge polarity. The imaging members as indicated herein are in embodiments sensitive in the wavelength region of, for example, from about 500 to about 900 nanometers, and in particular from about 650 to about 850 nanometers, thus diode lasers can be selected as the light source. Moreover, the imaging members of this invention are useful in color xerographic applications, particularly high-speed color 20 copying and printing processes.

## PRIOR ART

Layered photoresponsive imaging members have been described in numerous U.S. patents, such as U.S. Pat. No. 4,265,990, the disclosure of which is totally incorporated herein by reference, wherein there is illustrated an imaging member comprised of a photogenerating layer, and an aryl amine hole transport layer. Examples of photogenerating layer components include trigonal selenium, metal phthalocyanines, vanadyl phthalocyanines, and metal free phthalocyanines. Additionally, there is described in U.S. Pat. No. 3,121,006, the disclosure of which is totally incorporated herein by reference, a composite xerographic photoconductive member comprised of finely divided particles of 30 a photoconductive inorganic compound dispersed in an electrically insulating organic resin binder.

The use of perylene pigments as photoconductive substances is also known. There is thus described in Hoechst European Patent Publication 0040402, DE3019326, filed 40 May 21, 1980, the use of N,N'-disubstituted perylene-3,4, 9,10-tetracarboxyldiimide pigments as photoconductive substances. Specifically, there is, for example, disclosed in this publication N,N'-bis(3-methoxypropyl)perylene-3,4,9, 10-tetracarboxyl-diimide dual layered negatively charged 45 photoreceptors with improved spectral response in the wavelength region of 400 to 700 nanometers. A similar disclosure is presented in Ernst Gunther Schlosser, Journal of Applied Photographic Engineering, Vol. 4, No. 3, page 118 (1978). There are also disclosed in U.S. Pat. No. 3,871,882, the 50 disclosure of which is totally incorporated herein by reference, photoconductive substances comprised of specific perylene-3,4,9,10-tetracarboxylic acid derivative dyestuffs. In accordance with this patent, the photoconductive layer is preferably formed by vapor depositing the dyestuff in a 55 vacuum. Also, there are disclosed in this patent dual layer photoreceptors with perylene-3,4,9,10-tetracarboxylic acid diimide derivatives, which have spectral response in the wavelength region of from 400 to 600 nanometers. Further, in U.S. Pat. No. 4,555,463, the disclosure of which is totally 60 incorporated herein by reference, there is illustrated a layered imaging member with a chloroindium phthalocyanine photogenerating layer. In U.S. Pat. No. 4,587,189, the disclosure of which is totally incorporated herein by reference, there is illustrated a layered imaging member with, for example, a perylene, pigment photogenerating component. Both of the aforementioned patents disclose an aryl amine component, such as N,N'-diphenyl-N,N'-bis(3-methyl

phenyl)-1,1'-biphenyl-4,4'-diamine dispersed in a polycarbonate binder, as a hole transport layer. The above components, such as the photogenerating compounds, and the aryl amine charge transport can be selected for the imaging members of the present invention in embodiments thereof.

In U.S. Pat. No. 4,921,769, the disclosure of which is totally incorporated herein by reference, there are illustrated photoconductive imaging members with blocking layers of certain polyurethanes. Advantages of the hole blocking layer of the present invention over that of the '769 patent include, for example, excellent resistance to solvent degradation, superior electron transport and hole blocking, and ease of fabrication of the blocking layers, and wherein the blocking layer can be comprised of a crosslinked polymer network impregnated with a water-miscible hydroxy-functionalized polymer, thus enabling the addition of water to the blocking layer coating solution without causing, or minimizing phase separation during the coating process. Water can be an important reagent in alkoxy silane condensation reactions.

#### SUMMARY OF THE INVENTION

It is a feature of the present invention to provide imaging members with many of the advantages illustrated herein such as a rapid curing of the hole blocking layer during device fabrication, for example of about equal to, or less than about one minute, for example from about 5 to about 60 seconds, and which layer prevents, or minimizes dark injection, and wherein the resulting photoconducting members possess, for example, excellent photoinduced discharge characteristics, cyclic and environmental stability and acceptable charge deficient spot levels arising from dark injection of charge carriers.

Another feature of the present invention relates to the provision of layered photoresponsive imaging members, which are responsive to near infrared radiation of from about 700 to about 900 nanometers.

It is yet another feature of the present invention to provide layered photoresponsive imaging members with a sensitivity to visible light, and which members possess improved coating characteristics, and wherein the charge transport molecules do not diffuse, or there is minimum diffusion thereof into the photogenerating layer.

Moreover, another feature of the present invention relates to the provision of layered photoresponsive imaging members with mechanically robust and solvent resistant hole blocking layers.

In a further feature of the present invention there are provided imaging members containing hole blocking polymer layers comprised of a crosslinked polysiloxane polymer network impregnated with a hydroxy-functionalized polymer, and photogenerating pigments of, for example, Type V hydroxygallium phthalocyanine.

Aspects of the present invention relate to a photoconductive imaging member comprised of a supporting substrate, a hole blocking layer thereover, a photogenerating layer and a charge transport layer, and wherein the hole blocking layer is comprised of a hydroxy-functionalized polymer intertwined in a crosslinked polysiloxane network generated from crosslinking an organosilane reagent represented by Formula (I) or (II) below, optionally in the presence of a suitable silane crosslinking catalyst of, for example, an organoamine of, for example, triethylamine or carboxylic acid of, for example, acetic acid



wherein R is alkyl with, for example, from about 1 to about 20 carbon atoms, or aryl with, for example, from about 6 to about 30 carbon atoms; R<sup>1</sup>, R<sup>2</sup>, and R<sup>3</sup> are each independently selected from the group consisting of, for example, alkoxy of, for example, from about 1 to about 12 carbon atoms, aryloxy of, for example, from about 6 to about 24 carbon atoms, acyloxy of, for example, from about 2 to about 20 carbon atoms, halide, cyano, amino, and the like.

In accordance with aspects of the present invention, there is provided a photoconductive imaging member comprised of a supporting substrate, a hole blocking layer thereover, a photogenerating layer, and a charge transport layer, and wherein the hole blocking layer is generated from crosslinking an organosilane (I) in the presence of a hydroxy-functionalized polymer (II)



wherein R is alkyl or aryl, R<sup>1</sup>, R<sup>2</sup>, and R<sup>3</sup> are each independently selected from the group consisting of alkoxy, aryloxy, acyloxy, halide, cyano, and amino; A and B are, respectively, divalent and trivalent repeating segments or units of polymer (II); D is a divalent linkage; x and y represent the mole fractions of the repeating units of A and B, respectively, with x being from, for example, about 0 to about 0.99, more specifically, from about 0.3 to about 0.7 and y being from about 0.01 to about 1, and more specifically, from about 0.1 to about 0.75, and wherein the sum of x+y is equal to about 1; an imaging or photoconductive member wherein the organosilane (I) is selected from the group consisting of methyltrichlorosilane, methyltrimethoxysilane, methyltriethoxysilane, ethyltrichlorosilane, ethyltrimethoxysilane, ethyltriethoxysilane, propyltrimethoxysilane, 3-aminopropyltrimethoxysilane, 3-aminopropyltriethoxysilane, and the like; an imaging member wherein A is selected from the group consisting of



and B is selected from the group consisting of



an imaging member wherein D is arylene, aryleneoxycarbonyl, or alkyleneoxycarbonyl; wherein polymer (III) of the following Formula is selected as the hydroxyfunctionalized polymer (II)



wherein R and R'' are independently selected from the group consisting of hydrogen, alkyl, aryl, halogen, and the like; R' is aryl, cyano, halogen, alkoxy carbonyl, aryloxycarbonyl; D is divalent linkage preferably selected from the group consisting of arylene, alkylene aryl, alkyleneoxycarbonyl, aryleneoxycarbonyl, alkylene aryl oxycarbonyl; a and b are mole fractions of the repeating units of the polymer such that the sum of a+b=1; an imaging member wherein a is from about 0 to about 0.99, and b is from 0.01 to about 1 and wherein a+b=1; an imaging member wherein R and R'' are independently selected from hydrogen and alkyl, such as methyl, and R' is alkoxy carbonyl; an imaging member wherein R' is methoxycarbonyl, ethoxycarbonyl, propoxycarbonyl, or butoxycarbonyl; an imaging member wherein D is alkyleneoxycarbonyl or alkylene aryl oxycarbonyl; an imaging member wherein  $M_n$ , number average molecular weight of (III) is, for example, from about 1,000 to about 50,000, and  $M_w$ , weight average molecular weight is, for example, from about 10,000 to about 200,000; an imaging member wherein  $M_n$  of (III) ranges from about 5,000 to about 20,000, and  $M_w$  ranges from about 15,000 to about 75,000; an imaging member wherein organosilane (I) is selected from the group consisting of methyltrichlorosilane, methyltrimethoxysilane, methyltriethoxysilane, ethyltrichlorosilane, ethyltrimethoxysilane, ethyltriethoxysilane, propyltrimethoxysilane, 3-aminopropyltrimethoxysilane, 3-aminopropyl triethoxysilane, and the like; an imaging member wherein the organosilane (I) is 3-aminoalkyltrialkoxysilane; an imaging member wherein the organosilane (I) is 3-aminopropyltrialkoxysilane; an imaging member wherein the organosilane (I) is 3-aminopropyltrimethoxysilane or 3-aminopropyltriethoxysilane; an imaging member wherein alkyl contains from 1 to about 15 carbon atoms; an imaging member wherein alkyl contains from about 1 to about 10 carbon atoms; an imaging member wherein alkoxy contains from 1 to about 10 carbon atoms; an imaging member wherein the hydroxy-functionalized polymer (III) is selected from the group consisting of (III-a) through (III-h); a photoconductive imaging member wherein (III-a), (III-b), or (III-c) is selected, and wherein a and b are each from about 0.2 to about 0.8; a photoconductive imaging member wherein (III-d), (III-e), (III-f), (III-g), or (III-h) is selected, and wherein a and b are each from about 0.2 to about 0.8, and the sum thereof is about 1; a photoconductive imaging member wherein the organosilane (I) is

3-aminopropyltrimethoxysilane, 3-aminopropyl triethoxysilane, or mixtures thereof; a photoconductive imaging member wherein the hole blocking layer is of a thickness of about 0.001 to about 5 microns, or is of a thickness of about 0.1 to about 5 microns; a photoconductive imaging member comprised in the sequence of a supporting substrate, a hole blocking layer, an adhesive layer, a photogenerating layer and a charge transport layer; a photoconductive imaging member wherein the adhesive layer is comprised of a polyester with an  $M_w$  of about 70,000, and an  $M_n$  of about 35,000; a photoconductive imaging member wherein the supporting substrate is comprised of a conductive metal substrate; a photoconductive imaging member wherein the conductive substrate is aluminum, aluminized polyethylene terephthalate or titanized polyethylene; a photoconductive imaging member wherein the photogenerator layer is of a thickness of from about 0.05 to about 10 microns; a photoconductive imaging member wherein the charge, such as hole transport layer, is of a thickness of from about 10 to about 50 microns; a photoconductive imaging member wherein the photogenerating layer is comprised of photogenerating pigments dispersed in a resinous binder in an amount of from about 5 percent by weight to about 95 percent by weight; a photoconductive imaging member wherein the resinous binder is selected from the group consisting of polyesters, polyvinyl butyral, polycarbonates, polystyrene-b-polyvinyl pyridine, and polyvinyl formals; a photoconductive imaging member wherein the charge transport layers comprise aryl amine molecules; a photoconductive imaging member wherein the charge transport aryl amines are of the formula



wherein X is selected from the group consisting of alkyl and halogen, and wherein the aryl amine is dispersed in a resinous binder; a photoconductive imaging member wherein the aryl amine alkyl is methyl, wherein halogen is chlorine, and wherein the resinous binder is selected from the group consisting of polycarbonates and polystyrene; a photoconductive imaging member wherein the aryl amine is N,N'-diphenyl-N,N-bis(3-methyl phenyl)-1,1'-biphenyl-4,4'-diamine; a photoconductive imaging member further including an adhesive layer of a polyester with an  $M_w$  of about 70,000, and an  $M_n$  of about 35,000; a photoconductive imaging member wherein the photogenerating layer is comprised of metal phthalocyanines, or metal free phthalocyanines; a photoconductive imaging member wherein the photogenerating layer is comprised of titanyl phthalocyanines, perylenes, or hydroxygallium phthalocyanines; a photoconductive imaging member wherein the photogenerating layer is comprised of Type V hydroxygallium phthalocyanine; a method of imaging which comprises generating an electrostatic latent image on the imaging member illustrated herein, developing the latent image, and transferring the developed electrostatic image to a suitable substrate; a photoconductive imaging member wherein there is accomplished crosslinking in the presence of a catalyst such as, for example, a catalyst selected from the group consisting of carboxylic acids and amines; a photoconduc-

tive imaging member wherein acetic acid or an alkylamine is selected as the catalyst for the preparation of the hole blocking layer; a photoconductive imaging wherein the catalyst is propylamine or butylamine is selected; a photoconductive imaging wherein the catalyst for the preparation of the hole blocking layer is selected in the amount of about 0.01 to about 10 weight percent of the amount of organosilane (I); and a photoconductive imaging member comprised of a supporting substrate, a hole blocking layer thereover, a photogenerating layer, and a charge transport layer, and wherein the hole blocking layer is generated from crosslinking an organosilane (I) in the presence of a hydroxy-functionalized polymer (II)



wherein R is a suitable group or radical, such as alkyl with, for example, from about 1 to about 20 carbon atoms, aryl with, for example, from about 6 to about 30 carbon atoms and the like; R<sup>1</sup>, R<sup>2</sup>, and R<sup>3</sup> are, for example, independently selected from the group consisting of alkoxy with, for example, from about 1 to about 12 carbon atoms, aryloxy with, for example, from about 6 to about 24 carbon atoms, acyloxy with, for example, from about 2 to about 20 carbon atoms, halide, cyano, amino, and the like; A and B are, respectively, divalent and trivalent repeating segments of the polymer (II), for example, from about 2 to about 30 carbon atoms; D is a divalent linkage with, for example, from about 2 to about 30 carbon atoms such as arylene, aryleneoxycarbonyl, alkyleneoxycarbonyl, and the like; x and y are suitable mole fractions of the repeating units of A and B, respectively, wherein x is, for example, from about 0 to about 0.99, and y is, for example, from about 0.01 to about 1, and wherein the sum of x and y is about 1.

The hole blocking layers for the imaging members of the present invention are, for example, derived by crosslinking an organosilane reagent (I) in the presence of a hydroxy-functionalized polymer. The use of the hydroxy-functionalized polymer permits, for example, the addition of water into the hole blocking layer coating solution without, or minimizing phase separation. Water is usually present to permit the full crosslinking or curing of the organosilane (I) since usually the crosslinking reaction involves hydrolysis of (I) to provide the hydroxysilyl function (—Si—OH), which then undergoes self-condensation to provide a Si—O—Si bond as schematically represented in Scheme 1

Scheme 1



-continued



wherein R, R<sup>1</sup>, R<sup>2</sup>, and R<sup>3</sup> are substituents as indicated herein. The amount of crosslinking can vary depending on the reactants, for example; generally however, it is believed that from about 20 to about 95 percent of crosslinking can be accomplished.

Illustrative examples of organosilanes (I) or (I) include alkyl silanes, alkoxy silanes, amino silanes, alkylhalosilanes, aminoalkylalkoxysilanes, and more specifically for example, methyltrichlorosilane, methyltrimethoxysilane, methyltriethoxysilane, ethyltrichlorosilane, ethyltrimethoxysilane, ethyltriethoxysilane, propyltrimethoxysilane, 3-aminopropyltrimethoxysilane, 3-aminopropyltriethoxysilane, and the like.

In embodiments of the present invention, the hydroxy-functionalized polymer can be illustrated with reference to the general Formula (II)



wherein A and B are, respectively, divalent and trivalent repeating units of the polymer; D is a divalent linkage such as arylene, aryleneoxycarbonyl, alkyleneoxycarbonyl, and the like; m and n are the mole fractions of the repeating units of A and B, respectively, wherein x is, for example, from about 0 to about 0.99, and more specifically, from about 0.1 to about 0.9, and y is, for example, from about 0.01 to about 0.9, and wherein x+y is equal to 1.

65 Specific illustrative examples of A wherein x represents the number of repeating segments, such as from 1 to about 25, are

-continued



Specific illustrative examples of B are



and specific illustrative examples of D are



wherein p is, for example, a number of from about 2 to about 15;



The hydroxy-functionalized polymer that can be selected for the preparation of the hole blocking layer or layers of the present invention is illustrated with reference to Formula (III)



wherein R and R" are, for example, independently selected from the group consisting of hydrogen, alkyl, aryl, halogen, and the like; R' is aryl, cyano, halogen, alkoxy carbonyl, aryloxy carbonyl, and the like; D is, for example, selected from the group consisting of arylene, alkylene aryl, alkylene oxy carbonyl, arylene oxy carbonyl, alkylene aryl oxy carbonyl, and the like; a and b are as indicated herein, and more specifically, represent mole fractions of the repeating units of the polymer.

More specifically, the hydroxy-functionalized polymers (III) that are utilized in the hole blocking layers of the present invention are selected from the group consisting of polymers (III-a) through (III-h)



(III-b)



(III-c)



(III-d)



(III-e)

-continued



(III-f)

(III-g)

(III-h)

polymerization, the reaction mixture is diluted with a solvent, such as toluene or tetrahydrofuran, and poured into, for example, hexane to precipitate the polymer product. The latter is collected by filtration and dried in vacuo to provide polymer (III), which is characterized by gel permeation chromatography (GPC), and other relevant spectroscopic techniques such as IR and NMR spectroscopy:

Scheme 2



wherein a is from about 0 to about 0.99, and b is from about 0.01 to about 1.0, and wherein the sum of a and b is equal to 1.

Polymer (III) that can be utilized in the hole blocking layers of the photoconductive imaging members of the present invention can be prepared by free radical polymerization according to Scheme 2 wherein the substituents are as illustrated herein. Specifically, this polymer can be prepared by polymerization of a mixture of vinyl monomers (IV) and (V) in the presence of a suitable radical initiator such as benzoyl peroxide, 2,2'-azobis(2-methylpropanenitrile), and the like. The polymerization is generally accomplished in an inert solvent such as toluene, benzene, tetrahydrofuran, chloroform, or the like at a temperature of between about 30° C. to about 120° C. A specific preparative procedure for polymer (III) is as follows. A mixture of monomers (IV) and (V) in effective molar equivalent amounts and a solvent, such as toluene or tetrahydrofuran, are first charged to a reactor. The mixture is stirred at a temperature ranging, for example, from ambient to about 70° C. for about 5 to 30 minutes. Subsequently, an initiator, such as 2,2'-azobis(2-methylpropanenitrile), is added and the mixture is heated at about 50° C. to about 100° C. for a suitable period of time, for example from 1 to about 24 hours to complete the polymerization. After the

30 Specific embodiments of the present invention relate to a photoconductive imaging member wherein the hole blocking layer is of a thickness of about 0.001 to about 5 microns; a photoconductive imaging member wherein the hole blocking layer is of a thickness of about 0.1 to about 5 microns; a photoconductive imaging member wherein the blocking polymer is derived from a hydroxy-functionalized polymer 35 (II) and an organosilane (I) selected from the group consisting of alkylhalosilanes, alkylalkoxysilanes, aminoalkylsilanes, and the like, such as methyltrichlorosilane, methyltrimethoxysilane, methyltriethoxysilane, ethyltrichlorosilane, 40 ethyltrimethoxysilane, ethyltriethoxysilane, propyltrimethoxysilane, 3-aminopropyltrimethoxysilane, 3-aminopropyl triethoxysilane, and the like; a photoconductive imaging member wherein the organosilane (I) is 45 3-aminopropyltrimethoxysilane or 3-aminopropyl triethoxysilane; a photoconductive imaging member comprised in the following sequence of a supporting substrate, a hole blocking polymer network layer prepared from organosilane (I) and polymer (II) as illustrated herein, an adhesive layer, a photogenerating layer and a charge transport layer; a 50 photoconductive imaging member wherein the adhesive layer is comprised of a polyester with an  $M_w$  of, for example, from about 20,000 to about 100,000, and more specifically, about 35,000, and an  $M_n$  of from about 10,000 to 50,000, and more specifically, about 14,000; a photoconductive imaging member wherein the supporting substrate is comprised of a conductive metal substrate; a photoconductive imaging member wherein the conductive substrate is aluminum, aluminized or titanized polyethylene terephthalate belt (MYLAR®); a photoconductive imaging member 55 wherein the photogenerator layer is of a thickness of from about 1 to about 10 microns; a photoconductive imaging member wherein the transport layer is of a thickness of from about 10 to about 75 microns; a photoconductive imaging member wherein the photogenerating layer is comprised of photogenerating pigments dispersed in a resinous binder in an amount of from about 10 percent by weight to about 95 percent by weight; a photoconductive imaging member 60

wherein the resinous binder is selected from the group consisting of polyesters, polyvinyl butyral, polycarbonates, polystyrene-b-polyvinyl pyridines, and polyvinyl formals; a photoconductive imaging member wherein the charge transport layer comprises aryl amine molecules; a photoconductive imaging member wherein the aryl amines are of the formula



wherein X is selected from the group consisting of alkyl and halogen, and wherein the aryl amine is dispersed in a highly insulating and transparent resinous binder; a photoconductive imaging member wherein the arylamine alkyl contains from about 1 to about 12 carbon atoms; a photoconductive imaging member wherein the arylamine alkyl contains from 1 to about 5 carbon atoms; a photoconductive imaging member wherein the arylamine alkyl is methyl, wherein halogen is chloride, and wherein the resinous binder is selected from the group consisting of polycarbonates and polystyrenes; a photoconductive imaging member wherein the aryl amine is N,N'-diphenyl-N,N-bis(3-methylphenyl)-1,1'-biphenyl-4,4'-diamine; a photoconductive imaging member further including an adhesive layer of a polyester with an  $M_w$  of about 70,000, and an  $M_n$  of from about 25,000 to about 50,000, and more specifically about 35,000; a photoconductive imaging member wherein the photogenerating layer is comprised of metal phthalocyanines, metal free phthalocyanines or mixtures thereof; a photoconductive imaging member wherein the photogenerating layer is comprised of titanyl phthalocyanines, perylenes, such as BZP, or hydroxygallium phthalocyanines; a photoconductive imaging member wherein the photogenerating layer is comprised of Type V hydroxygallium phthalocyanine; a method of imaging which comprises generating an electrostatic latent image on the imaging member, developing the latent image with a know dry toner, and transferring the developed electrostatic image to a suitable substrate; a photoconductive imaging member wherein the blocking layer is derived from the reaction of organosilane (I) in the presence of hydroxy-functionalized polymer (II) and an optional catalyst selected from the group consisting of carboxylic acids and amines; a photoconductive imaging member wherein acetic acid or an alkylamine is selected as the catalyst; an imaging member wherein an interpenetrating hydroxy-functionalized polymer (II)/polysiloxane network is selected as a hole blocking layer, and is generated from the hydrolysis and polycondensation of organosilane (I) in the presence of (II); and imaging members comprised of a supporting substrate, an interpenetrating polysiloxane/hydroxy-functionalized polymer network blocking layer, thereover, a photogenerating layer of, for example, hydroxygallium phthalocyanine, and a charge transport layer.

Illustrative examples of monomer (IV) selected for the preparation of polymer (III) include, for example, acrylonitrile, vinyl chloride, styrene, methyl styrene, chlorostyrene, acrylic and methacrylic esters such as methyl acrylate, ethyl acrylate, propyl acrylate, butyl acrylate, methyl methacrylate, ethyl methacrylate, propyl methacrylate, butyl methacrylate, phenyl acrylate, phenyl

methacrylate, and the like. Illustrative examples of monomer (V) include, for example, 2-hydroxyethyl methacrylate, hydroxypropyl methacrylate, 2-hydroxyethyl acrylate, hydroxypropyl acrylate, 4-hydroxybutyl acrylate, 2-allyphenol, allyl alcohol, 2-allyl-6-methoxyphenol, 4-allyl-2-methoxyphenol, 4-allyl-2,6-dimethoxyphenol, and the like.

Specifically, the preparation of the hole blocking layers of the present invention involves coating a solution of polymer (III), organosilane (I), optional catalyst, and water in a suitable solvent onto a supporting substrate. The coated layer is then thermally dried and cured at elevated temperatures. The curing or crosslinking can generally be accomplished at, for example, about 40° C. to about 200° C., and preferably from about 80° C. to about 150° C. for a suitable time period such as from about 0.1 minute to about 2 hours. The crosslinking processes, as schematically illustrated in Scheme 1, involves the hydrolysis of the silyl groups of organosilane (I) to the corresponding hydroxysilane functions, followed by condensation to form the siloxane (Si—O—Si) bonds. It is preferred that water, for example from about 0.001 to about 10 weight percent, be present in the coating solution to fully effect the hydrolysis for the crosslinking reaction. Trace amounts of water, such as for example about 0.01 percent by weight of solvent that are present in the coating solvents, may often be sufficient to induce the hydrolysis reaction. Additionally, curing or crosslinking of the coated blocking layers may also be induced to occur by humidification via exposing to a moist atmosphere prior to or during thermal treatment.

Illustrative examples of substrate layers selected for the imaging members of the present invention can be opaque or substantially transparent, and may comprise any suitable material having the requisite mechanical properties. Thus, the substrate may comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass or the like. The substrate may be flexible, seamless, or rigid, and may have a number of many different configurations, such as for example a plate, a cylindrical drum, a scroll, an endless flexible belt, and the like. In one embodiment, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

The thickness of the substrate layer depends on many factors, including economical considerations, thus this layer may be of substantial thickness, for example over 3,000 microns, or of minimum thickness providing there are no significant adverse effects on the member. In embodiments, the thickness of this layer is from about 75 microns to about 300 microns.

The photogenerating layer, which can be comprised of hydroxygallium phthalocyanine Type V, is in embodiments comprised of, for example, about 50 weight percent of the Type V and about 50 weight percent of a resin binder like polystyrene/polyvinylpyridine. The photogenerating layer can contain known photogenerating pigments, such as metal phthalocyanines, metal free phthalocyanines, hydroxygallium phthalocyanines, perylenes, especially bis (benzimidazo)perylene, titanyl phthalocyanines, and the

15

like, and more specifically vanadyl phthalocyanines, Type V hydroxygallium phthalocyanines, and inorganic components such as selenium, especially trigonal selenium. The photogenerating pigment can be dispersed in a resin binder similar to the resin binders selected for the charge transport layer, or alternatively no resin binder is needed. Generally, the thickness of the photogenerator layer depends on a number of factors, including the thicknesses of the other layers and the amount of photogenerator material contained in the photogenerating layers. Accordingly, this layer can be of a thickness of, for example, from about 0.05 micron to about 10 microns, and more specifically, from about 0.25 micron to about 2 micron when, for example, the photogenerator compositions are present in an amount of from about 30 to about 75 percent by volume. The maximum thickness of this layer in embodiments is dependent primarily upon factors, such as photosensitivity, electrical properties and mechanical considerations. The photogenerating layer binder resin, present in various suitable amounts, for example from about 1 to about 50, and more specifically, from about 1 to about 10 weight percent, may be selected from a number of known polymers such as poly(vinyl butyral), poly(vinyl carbazole), polyesters, polycarbonates, poly(vinyl chloride), polyacrylates and methacrylates, copolymers of vinyl chloride and vinyl acetate, phenoxy resins, polyurethanes, poly(vinyl alcohol), polyacrylonitrile, polystyrene, and the like. It is desirable to select a coating solvent that does not substantially disturb or adversely effect the other previously coated layers of the device. Examples of solvents that can be selected for use as coating solvents for the photogenerator layers are ketones, alcohols, aromatic hydrocarbons, halogenated aliphatic hydrocarbons, ethers, amines, amides, esters, and the like. Specific examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The coating of the photogenerator layers in embodiments of the present invention can be accomplished with spray, dip or wire-bar methods such that the final dry thickness of the photogenerator layer is, for example, from about 0.01 to about 30 microns and more specifically from about 0.1 to about 15 microns after being dried at, for example, about 40° C. to about 150° C. for about 15 to about 90 minutes.

Illustrative examples of polymeric binder materials that can be selected for the photogenerator layer are as indicated herein, and include those polymers as disclosed in U.S. Pat. No. 3,121,006, the disclosure of which is totally incorporated herein by reference. In general, the effective amount of polymer binder that is utilized in the photogenerator layer ranges from about 0 to about 95 percent by weight, and preferably from about 25 to about 60 percent by weight of the photogenerator layer.

As optional adhesive layers usually in contact with the hole blocking layer, there can be selected various known substances inclusive of polyesters, polyamides, poly(vinyl butyral), poly(vinyl alcohol), polyurethane and polyacrylonitrile. This layer is, for example, of a thickness of from about 0.001 micron to about 1 micron. Optionally, this layer may contain effective suitable amounts, for example from about 1 to about 10 weight percent, conductive and non-conductive particles, such as zinc oxide, titanium dioxide, silicon nitride, carbon black, and the like, to provide, for example, in embodiments of the present invention further desirable electrical and optical properties.

16

Aryl amines selected for the charge, especially hole transporting layers, which generally are of a thickness of from about 5 microns to about 75 microns, and preferably of a thickness of from about 10 microns to about 40 microns, include molecules of the following formula



dispersed in a highly insulating and transparent polymer binder, wherein X is an alkyl group, a halogen, or mixtures thereof, especially those substituents selected from the group consisting of Cl and CH<sub>3</sub>.

Examples of specific aryl amines are N,N'-diphenyl-N,N'-bis(alkylphenyl)-1,1-biphenyl-4,4'-diamine wherein alkyl is selected from the group consisting of methyl, ethyl, propyl, butyl, hexyl, and the like; and N,N'-diphenyl-N,N'-bis(halophenyl)-1,1'-biphenyl-4,4'-diamine wherein the halo substituent is preferably a chloro substituent. Other known charge transport layer molecules can be selected, reference for example U.S. Pat. Nos. 4,921,773 and 4,464,450, the disclosures of which are totally incorporated herein by reference.

Examples of the highly insulating and transparent polymer binder materials for the transport layers include components, such as those described in U.S. Pat. No. 3,121,006, the disclosure of which is totally incorporated herein by reference. Specific examples of polymer binder materials include polycarbonates, acrylate polymers, vinyl polymers, cellulose polymers, polyesters, polysiloxanes, polyamides, polyurethanes and epoxies as well as block, random or alternating copolymers thereof. Preferred electrically inactive binders are comprised of polycarbonate resins having a molecular weight of from about 20,000 to about 100,000 with a molecular weight of from about 50,000 to about 100,000 being particularly preferred. Generally, the transport layer contains from about 10 to about 75 percent by weight of the charge transport material, and preferably from about 35 percent to about 50 percent of this material.

Also, included within the scope of the present invention are methods of imaging and printing with the photoresponsive devices illustrated herein. These methods generally involve the formation of an electrostatic latent image on the imaging member, followed by developing the image with a toner composition comprised, for example, of thermoplastic resin, colorant, such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same steps with the exception that the exposure step can be accomplished with a laser device or image bar.

The following Examples are being submitted to illustrate embodiments of the present invention. These Examples are intended to be illustrative only and are not intended to limit the scope of the present invention. Also, parts and percentages are by weight unless otherwise indicated. Comparative Examples and data are also provided.

## 17

## EXAMPLE I

Synthesis of Polymer (III-a) With  $a=0.30$ ,  $b=0.70$ :

To a 1 liter three-neck round-bottomed flask, under a nitrogen blanket, were added 15.02 grams of methyl methacrylate, 45.55 grams of 2-hydroxyethyl methacrylate, 300 milliliters of tetrahydrofuran and 85 milliliters of ethanol. The resulting mixture was stirred at about 30° C. for 10 minutes, followed by the addition of 0.632 gram of 2,2'-azobis(isobutyronitrile) initiator. The mixture resulting was subsequently stirred and refluxed for 24 hours at temperature of about 85° C. The resulting polymer solution was diluted with 500 milliliters of tetrahydrofuran at room temperature, about 25° C. throughout, and was then added into 5,000 milliliters of hexane with stirring to precipitate the polymer product. The solid product, polymer (III-a), was collected by filtration and dried at room temperature in vacuo for 24 hours to provide 55.7 grams (91 percent) of polymer (III-a). The polymer displayed an  $M_w$  of 35,704 and an  $M_n$  of 15,504, both as measured by GPC.

## EXAMPLE II

Synthesis of Polymer (III-a) With  $a=0.70$  and  $b=0.30$ :

This polymer was prepared in accordance with the procedure of Example I except that 35.04 grams of methyl methacrylate, 19.52 grams of 2-hydroxyethyl methacrylate, 400 milliliters of tetrahydrofuran, and 0.657 grams of 2,2'-azobis(isobutyronitrile) initiator were utilized. The yield was 50 grams (91.6 percent).

The polymer displayed an  $M_w$  of 29,620 and an  $M_n$  of 13,703 as measured by GPC.

## EXAMPLE III

Synthesis of Polymer (III-a) With  $a=50$  and  $b=0.50$ :

This polymer was prepared in accordance with the procedure of Example II except that 25.03 grams of methyl methacrylate, 32.54 grams of 2-hydroxyethyl methacrylate, 300 milliliters of tetrahydrofuran, 85 milliliters of ethanol, and 0.63 gram of 2,2'-azobis(isobutyronitrile) initiator were utilized. The yield was 52.4 grams (91.0 percent).

The polymer displayed an  $M_w$  of 34,425 and an  $M_n$  of 13,738 as measured by GPC.

## EXAMPLE IV

An illustrative photoresponsive imaging device incorporating the blocking layer of the present invention was fabricated as follows.

A 75 micron thick titanized MYLAR® substrate was coated by known draw bar techniques with a hole blocking layer from a solution of 1.6 grams of polymer (III-a) of Example I and 0.4 gram of 3-aminopropyl trimethoxysilane in 8 grams of a 96.0/1.5/2.5 (by weight percent) of a mixture of ethanovacetic acid/water. After drying at 135° C. for 1 minute, a blocking layer (HBL) of about 3.4 to about 3.9 microns was obtained. Overcoated on the top of the blocking layer was a 0.05 micron thick adhesive layer prepared from a solution of 2 weight percent of an E.I. DuPont 49K (49,000) polyester in dichloromethane. A 0.2 micron photogenerating layer was subsequently coated on top of the adhesive layer from a dispersion of hydroxy gallium phthalocyanine Type V (0.46 gram) and a polystyrene-b-polyvinylpyridine block copolymer (0.48 gram) in 20 grams of toluene, followed by drying at 10° C. for 10 minutes. Subsequently, a 25 micron charge transport layer (CTL) was coated on top of the photogenerating layer from a solution of N,N'-diphenyl-N,N'-bis(3-methyl phenyl)-1,1'-biphenyl-4,4'-diamine (2.64 grams) and a polycarbonate (3.5 grams) in 40 grams of dichloromethane.

A control device was also prepared in a similar manner without the above blocking layer.

The xerographic electrical properties of the imaging members can be determined by known means, including as

## 18

indicated herein electrostatically charging the surfaces thereof with a corona discharge source until the surface potentials, as measured by a capacitively coupled probe attached to an electrometer, attained an initial value  $V_o$  of about -800 volts. After resting for 0.5 second in the dark, the charged members attained a surface potential of  $V_{ddp}$ , dark development potential. Each member was then exposed to light from a filtered Xenon lamp with a XBO 150 watt bulb, thereby inducing a photodischarge which resulted in a reduction of surface potential to a  $V_{bg}$  value, background potential. The percent of photodischarge was calculated as  $100 \times (V_{ddp} - V_{bg})/V_{ddp}$ . The desired wavelength and energy of the exposed light was determined by the type of filters placed in front of the lamp. The monochromatic light photosensitivity was determined using a narrow band-pass filter.

The following table summarizes the electrical performance of these devices, which shows the effective blockage of dark charge injection by the hole blocking layer (HBL) of the present invention. Specifically, while the dark development potential ( $V_{ddp}$ ), the half discharge exposure energy ( $E_{1/2}$ ), and the residual voltage are similar for the control device and the device of the present invention, the dark decay, which measures the dark conductivity related to hole injection into the photogenerator layer, of the device of the present invention is significantly lower than that of the control device or photoconductive imaging member.

| Device #                       | CTL<br>( $\mu$ m) | V <sub>ddp</sub><br>(V) | E <sub>1/2</sub><br>ergs/cm <sup>2</sup> | Dark Decay<br>(V @ 500 ms) | V <sub>r</sub><br>(V) |
|--------------------------------|-------------------|-------------------------|------------------------------------------|----------------------------|-----------------------|
| Control Device                 | 25.0              | 813                     | 1.54                                     | 19.5                       | 0-4                   |
| Without HBL                    |                   |                         |                                          |                            |                       |
| Device with 3.4-3.9<br>$\mu$ m | 24.9              | 802                     | 1.36                                     | 5.9                        | 0-2                   |
| Crosslinked Siloxane<br>HBL    |                   |                         |                                          |                            |                       |

## EXAMPLE V

A photoresponsive imaging device with a hole blocking layer of the present invention was fabricated in accordance with the procedure of Example IV except that the blocking layer was prepared from a solution of 1 gram of polymer (III-a) of Example I and 1 gram of 3-aminopropyltrimethoxysilane in 8 grams of a 90.0/3.8/6.2 (by weight percent) mixture of ethanol/acetic acid/water. After drying at 135° C. for 1 minute, a hole blocking layer (HBL) of about 2.5 to 3.3 microns was obtained. The following table summarizes the electrical performance of this device.

| Device #                       | CTL<br>( $\mu$ m) | V <sub>ddp</sub><br>(V) | E <sub>1/2</sub><br>ergs/cm <sup>2</sup> | Dark Decay<br>(V @ 500 ms) | V <sub>r</sub><br>(V) |
|--------------------------------|-------------------|-------------------------|------------------------------------------|----------------------------|-----------------------|
| Control Device<br>without HBL  | 25.0              | 813                     | 1.54                                     | 19.5                       | 0-4                   |
| Device with 2.5-3.3<br>$\mu$ m | 24.3              | 807                     | 1.40                                     | 8.8                        | 0-5                   |
| Crosslinked Siloxane<br>HBL    |                   |                         |                                          |                            |                       |

## EXAMPLE VI

A photoresponsive imaging device with a hole blocking layer derived from polymer (III-a) of Example III was prepared in accordance with the procedure of Example V.

The HBL thickness was about 2 to 2.3 microns, and was, more specifically, prepared from a solution of 1 gram of polymer (III-a) of Example III and 1 gram of 3-aminopropyltrimethoxysilane in 8 grams of a 90.0/3.8/6.2 (by weight percent) mixture of ethanovacetic acid/water. After drying at 135° C. for 1 minute, a hole blocking layer (HBL) of about 2 to 2.3 microns was obtained. The following table summarizes the electrical performance of this device.

| Device #                                                      | CTL<br>( $\mu$ m) | Vddp<br>(V) | $E_{1/2}$<br>ergs/cm <sup>2</sup> | Dark Decay<br>(V @ 500 ms) | V <sub>r</sub><br>(V) |
|---------------------------------------------------------------|-------------------|-------------|-----------------------------------|----------------------------|-----------------------|
| Control Device<br>without HBL                                 | 25.0              | 813         | 1.54                              | 19.5                       | 0-4                   |
| Device with 2.0-2.3<br>$\mu$ m<br>Crosslinked Siloxane<br>HBL | 25.4              | 805         | 1.46                              | 10.3                       | 0-5                   |

Other embodiments and modifications of the present invention may occur to those skilled in the art subsequent to a review of the information presented herein; these embodiments and modifications, as well as equivalents thereof, are also included within the scope of this invention.

What is claimed is:

1. A photoconductive imaging member comprised of an optional supporting substrate, a hole blocking layer thereover, a photogenerating layer, and a charge transport layer, and wherein the hole blocking layer is generated from crosslinking an organosilane (I) in the presence of a hydroxy-functionalized polymer (II)



wherein R is alkyl or aryl, R<sup>1</sup>, R<sup>2</sup>, and R<sup>3</sup> are independently selected from the group consisting of alkoxy, aryloxy, acyloxy, halide, cyano, and amino; A and B are respectively divalent and trivalent repeating units of polymer (II); D is a divalent linkage; x and y represent the mole fractions of the repeating units of A and B, respectively, and wherein x is from about 0 to about 0.99, and y is from about 0.01 to about 1, and wherein the sum of x+y is equal to about 1.

2. An imaging member in accordance with claim 1 wherein said organosilane is selected from the group consisting of methyltrichlorosilane, methyltrimethoxysilane, methyltriethoxysilane, ethyltrichlorosilane, ethyltrimethoxysilane, ethyltriethoxysilane, propyltrimethoxysilane, 3-aminopropyltrimethoxysilane, and 3-aminopropyltriethoxysilane.

3. An imaging member in accordance with claim 1 wherein A is selected from the group consisting of

5



10 wherein x represents the number of repeating segments, and B is selected from the group consisting of



15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695

21

12. An imaging member in accordance with claim 1 wherein said organosilane (I) is 3-aminoalkyltrialkoxysilane.

13. An imaging member in accordance with claim 1 wherein said organosilane (I) is 3-aminopropyltrialkoxysilane.

14. An imaging member in accordance with claim 1 wherein said organosilane (I) is 3-aminopropyltrimethoxysilane or 3-aminopropyltriethoxysilane.

15. An imaging member in accordance with claim 14 wherein alkyl contains from about 1 to about 15 carbon atoms, or wherein alkyl contains from about 1 to about 10 carbon atoms, and wherein alkoxy contains from about 1 to about 10 carbon atoms.

16. An imaging member in accordance with claim 5 wherein said hydroxy-functionalized polymer (III) is selected from the group consisting of (III-a) through (III-h).

17. A photoconductive imaging member in accordance with claim 16 wherein (III-a), (III-b), or (III-c) is selected, and wherein a and b are each from about 0.2 to about 0.8, or wherein (III-d), (III-e), (III-f), (III-g), or (III-h) is selected, and wherein a and b are each from about 0.2 to about 0.8.

18. A photoconductive imaging member in accordance with claim 16 wherein said organosilane (I) is 3-aminopropyltrimethoxysilane, or 3-aminopropyltriethoxysilane.

19. A photoconductive imaging member in accordance with claim 1 wherein said hole blocking layer is of a thickness of about 0.001 to about 5 microns.

20. A photoconductive imaging member in accordance with claim 1 wherein said hole blocking layer is of a thickness of about 0.1 to about 5 microns, and optionally wherein said layer is a two-phase layer wherein a hydroxy polymer is dispersed in a crosslinked polymer matrix.

21. A photoconductive imaging member in accordance with claim 1 comprised in the following sequence of a supporting substrate, said hole blocking layer, an adhesive layer, a photogenerating layer, and wherein the charge transport layer is a hole transport layer.

22. A photoconductive imaging member in accordance with claim 21 wherein the adhesive layer is comprised of a polyester with an  $M_w$  of about 70,000, and an  $M_n$  of about 35,000.

23. A photoconductive imaging member in accordance with claim 1 wherein the supporting substrate is comprised of a conductive metal substrate, and optionally which substrate is aluminum, aluminized polyethylene terephthalate or titanized polyethylene terephthalate.

24. A photoconductive imaging member in accordance with claim 1 wherein said photogenerator layer is of a thickness of from about 0.05 to about 10 microns, and wherein said transport layer is of a thickness of from about 10 to about 50 microns.

25. A photoconductive imaging member in accordance with claim 1 wherein the photogenerating layer is comprised of photogenerating pigments dispersed in a resinous binder in an optional amount of from about percent by weight to about 95 percent by weight, and optionally wherein the

22

resinous binder is selected from the group consisting of polyesters, polyvinyl butyral, polycarbonates, polystyrene-b-polyvinyl pyridine, and polyvinyl formals.

26. A photoconductive imaging member in accordance with claim 1 wherein the charge transport layer comprises aryl amines, and which aryl amines are optionally of the formula



wherein X is selected from the group consisting of alkyl and halogen, and wherein the aryl amine is dispersed in a highly insulating and transparent resinous binder.

27. A photoconductive imaging member in accordance with claim 26 wherein alkyl contains from about 1 to about 10 carbon atoms, or wherein alkyl contains from 1 to about 5 carbon atoms, or optionally wherein alkyl is methyl, wherein halogen is chlorine, and wherein the resinous binder is selected from the group consisting of polycarbonates and polystyrenes.

28. A photoconductive imaging member in accordance with claim 27 wherein the aryl amine is N,N'-diphenyl-N,N-bis(3-methyl phenyl)-1,1'-biphenyl-4,4'-diamine.

29. A photoconductive imaging member in accordance with claim 1 wherein the photogenerating layer is comprised of metal phthalocyanines, or metal free phthalocyanines.

30. A photoconductive imaging member in accordance with claim 1 wherein the photogenerating layer is comprised of titanyl phthalocyanines, perylenes, or hydroxygallium phthalocyanines.

31. A photoconductive imaging member in accordance with claim 1 wherein the photogenerating layer is comprised of Type V hydroxygallium phthalocyanine.

32. A method of imaging which comprises generating an electrostatic latent image on the imaging member of claim 1, developing the latent image, and transferring the developed electrostatic image to a suitable substrate.

33. A photoconductive imaging member in accordance with claim 1 wherein there is accomplished a crosslinking in the presence of a catalyst optionally selected from the group consisting of carboxylic acids and amines.

34. A photoconductive imaging member in accordance with claim 33 wherein acetic acid or an alkylamine is selected as the catalyst.

35. A photoconductive imaging member in accordance with claim 33 wherein propylamine or butylamine is selected.

36. A photoconductive imaging member in accordance with claim 33 wherein the catalyst is selected in the amount of about 0.01 to about 10 weight percent of the amount of organosilane (I).

\* \* \* \* \*